

Patented Jan. 14, 1930

## Cross Reference

1,743,551

## UNITED STATES PATENT OFFICE

JAMES KEETH, OF SPOKANE, WASHINGTON

## PLASTIC COMPOSITION

No Drawing.

Application filed April 9, 1926. Serial No. 100,980.

106-75

My present invention relates to a new and improved plastic composition for heat insulating, such as coverings for steam boilers, steam and refrigerator pipes and for refrigerators, as well as for plastering walls of dwellings, apartment houses, hotels and other building structures for securing heat proof and sound proof walls.

The composition of my invention may be used as a plaster and applied in the customary manner, or it may be made up if desired in sheets or boards, or in tubular sections, and applied according to existing modes for using such articles in building structures or as coverings for pipes.

The plastic composition consists essentially of a plaster obtained by thoroughly mixing and intermingling finely powdered jefferisite and paper or wood pulp, and the composition also contemplates the use of a binder and surface-hardener as sodium silicate or an alkaline salt.

Jefferisite, as raw material in its natural state, is found and mined in sheets or books of various sizes, which are comparatively light in weight in proportion to their size, and after roasting or baking in an oven or other suitable place for heat treatment, a given weight of the material expands or increases in size, and decreases in weight as the moisture is removed therefrom. After exfoliation by baking or roasting the jefferisite retains its book or leaf formation, but the books are so light and fragile that the material may be crushed to powder form or pulverized into a flaky mass between the fingers of the hand.

Thus the roasted jefferisite is finely rendered or comminuted in a suitable mill to form a fine flaky powder which has a color blending from a gold to a silver hue. This material as thus prepared is especially adapted for use as a heat insulating element in the plastic composition, and is used in my plaster for that purpose.

The pulp, which may be obtained by macerating either waste paper or prepared wood, is used as a filler and reinforcing element for the plastic composition.

In the process of preparing the plaster or

plastic composition, after the jefferisite has been exfoliated by roasting or baking and finely comminuted, it is placed with the pulp in a suitable vessel and the required quantity of water added. The materials are then thoroughly agitated, stirred, and mixed to thoroughly incorporate the elements into a plastic mass or composition, which is then ready for application in plastic condition as a substitute for various heat insulating materials used on hot or cold pipes such as steam and hot water pipes or refrigerator pipes, and on furnaces, steam boilers, etc. The two materials may be used in approximately the same relative proportions, which may be varied within limits, when the plaster is to be used as a covering or heat insulator alone. The plaster is applied to the surface to be coated or covered by the use of suitable tools or implements, or may be applied by hand and smoothed on, and as it possesses the quality of adhesion to a high degree, it is free from cracks or other defects when dry.

In color the dry covering presents an appearance of a light gold hue, and the structure of the covering, which has a cellular formation, is comparatively light in weight (thus only slightly increasing the weight of a covered pipe or other tubular structure) and forms an excellent insulating medium against the transmission of heat.

In the preparation of the plastic composition for use as a wall plaster for use on laths in dwellings and other building structures, or as a plaster board for that purpose, in addition to its qualities as a heat insulator, the plastic composition also forms a sound proof material against the transmission of sound waves. To provide this quality in the plastic material a binder and surface-hardener, such as sodium silicate, is in some instances added to the two first mentioned ingredients as they are being mixed, and the binder is thoroughly incorporated and mixed with the wet ingredients to form a plastic material.

In this condition the plaster or plastic composition may with facility be manipulated by the use of a trowel or other implement and applied to the lathing and spread or flowed

on in usual manner. When the wall thus prepared dries by evaporation of the moisture in the plastic material, the exposed surface of the wall is found to be hard and tough, while the interior or core of the wall is less hard. The surface presents a glazed appearance with a darker golden hue than that obtained in the mixture of jeffersite and pulp alone, and this surface can be used as the finished surface of the plastered wall, or a finishing coat of selected color may be added if desired.

This hard, glazed, or glassy appearing surface adds the sound-proof quality to the plastered wall, in addition to its heat insulating quality, and the hard glazed surface is instrumental in reflecting or deflecting sound waves that may strike it, which sound waves are thus prevented from being transmitted through the wall. These qualities as a heat-insulating wall and as a sound proof wall adapt the plastic composition or plaster especially for use in dwellings, hotels, apartments and other building structures where it is desirable to use sound proof material in the walls.

As an example of the formula used in the preparation of the heat-proof and sound proof plaster or plastic composition, the following proportions may be stated.

|                      | Per cent |
|----------------------|----------|
| Jeffersite           | 60       |
| Pulp (wood or paper) | 35       |
| Sodium silicate      | 5        |

These proportions may however be varied within limits to suit different conditions or uses to which the plastic composition is to be adapted.

Having thus fully described my invention, what I claim as new and desire to secure by Letters Patent is—

1. A plastic composition comprising exfoliated and pulverized jeffersite, a pulp filler, and a binder.
2. The process of forming a plastic composition which consists in exfoliating jeffersite by roasting, finely comminuting the exfoliated material, mixing said material with a pulp in the presence of water, and adding a binder material to the mixture.

In testimony whereof I affix my signature.

JAMES KEETH.

*Jeffersite is a kind of vermiculite from West Chester, Penna.*

(Glossary of Mining & Mineral Industry, U.S. Bureau Mines 1949 - p. 369)